

Dec. 18, 1928.

1,695,805

J. GATTI

WADDING AND BAT

Filed Feb. 2, 1928

*Fig. 1.*



*Fig. 2.*



*Fig. 3.*



*Fig. 4.*



INVENTOR:  
Joseph Gatti,  
BY Cha. M. C. Chapman/  
ATTORNEY

Patented Dec. 18, 1928.

1,695,805

# UNITED STATES PATENT OFFICE.

JOSEPH GATTI, OF NEW YORK, N. Y., ASSIGNOR TO GATTI SERVICE INCORPORATED, OF NEW YORK, N. Y., A CORPORATION OF NEW JERSEY.

## WADDING AND BAT.

Application filed February 2, 1928. Serial No. 251,270.

This invention relates to wadding, bats and batting of fibrous material, and particularly has reference to a wadding for clothing, quilts, spreads, covers, mattresses and similar articles and uses, and to bats or batting made of the said wadding adapted for use in upholstering, in cushions, as a filling, and for various other purposes such as linings for the various parts of automobile bodies.

Among the objects of my invention may be noted the following: to provide a wadding which is light and sanitary and capable of being compressed into small compass so as to be used for the linings of coats, for comforters, spreads, coverings of all sorts, for mattresses, etc.; to provide a wadding which is composed of wood-pulp and cotton-fiber, linters and other fibrous material thoroughly intermixed; to provide a durable and light wadding material adapted for many uses, and which is odorless, is economical to produce, and which can be readily compressed and will retain its form, when made into bats or batting, without the addition of a binder or material calculated to retain the folded parts in place and the folded material in form.

With the above objects in view, and others which will be detailed during the course of this description, my invention consists in the parts, features, elements and combinations thereof hereinafter described and claimed.

In order that my invention may be clearly understood, I have provided drawings wherein:

Figure 1 is a plan view of a portion of a strip of wadding illustrating my invention;

Figure 2 is an edge elevation of Figure 1, a part of the wadding being broken away at one end to show the intermixture of the pulp and fiber according to my invention;

Figure 3 is a perspective view of a piece of wadding formed into a bat by rolling the same so as to overlap the edges thereof; and

Figure 4 is a perspective view of a piece of wadding folded to make a bat of predetermined width and thickness and indefinite length.

Referring to the drawings, it will be seen that my product, whether it be merely a sheet of wadding, or wadding folded into such form as to constitute a bat, batting or filling, is composed of wood-pulp and cotton-

fiber or linters or other suitable fibers, intermixed with the wood-pulp. The quantity of fiber, in proportion to the wood-pulp, may be varied, and it will be understood that I do not restrict myself, in manufacturing my product, to any precise proportion of the fiber relatively to the wood-pulp. The proportions may differ materially according to the use to which the wadding is to be put. As a general rule, I employ short cotton-fiber, linters, or sugar cane fiber, which will act as a binder for the wood-pulp to hold the granules thereof together so as to constitute a substantial fabric. Certain kinds or grades of fiber may be used in greater quantity proportionally to the wood-pulp, other kinds or grades may be used in lesser quantity; but, according to my invention, a sufficient quantity of fiber must be used to form a binder for the wood-pulp mass.

The wadding can be made of indefinite width and length, and may be made of widths and thicknesses suitable for many different purposes. It will be very wide for quilts, comforters, mattresses, etc.; it will be narrower for linings for clothing, fillings for pillows, etc., and still narrower for surgical use, such as for broken members of the anatomy, in which instance it may be used in connection with splints, whether of wood or plaster. If used as a bat or batting, it will be rolled into the form shown in Figure 3, and, when so rolled, may be compressed so as to cause the layers of the bat to hold their form, thus avoiding the necessity of using a foreign substance, such as glue or other adhesive, to hold the overlapped portions together. The same is true of the form of bat shown in Figure 4, wherein the parts of the wadding are shown as folded so as to have three superposed layers, the layers being compressed so as to cause the bat to hold its form.

In Figures 1 and 2, I have shown a strip of my material to be used as a wadding, lining or filling, and the numeral 1 indicates generally such material. In Figure 2, at the point where the material has been broken away to illustrate the composition thereof, the dots 2 are intended to illustrate the granules of wood-pulp, while the curved lines 3 are intended to illustrate the fibers or linters intermixed with the wood-pulp granules and with each other, so as to operate as a binder between the fiber and pulp. From this it

will be seen that, when the fiber and pulp are intermixed thoroughly, the granules of the pulp foundation will be held intimately by the fibers, and, when the sheet of wadding is compressed for its various purposes, or for the purpose of giving it a desired thickness and solidity, the pulp and fiber will be more intimately related, giving to the sheet of material greater tensile strength.

10. If it is desired to provide the wadding or sheet material with glazed surfaces, I apply thereto a thin coat of limpid glucose and subject the material to pressure and heat so as to dry the coating upon the surfaces of 15 the material, this structure being indicated at 4 by the heavy line on the opposite surfaces of the strip.

When the sheet of wadding of Figure 1 is rolled to make a bat, the contiguous surfaces 20 5 of the material will frictionally hold, and under pressure, the bat will assume the form shown in Figure 3; or a bat can be also made by folding the sheet of Figure 1 into 25 several superposed layers and the contiguous surfaces 6 will be caused to hold by pressure, and the bat will assume the form of Figure 4. The greater the pressure the flatter the bat or the material; and by pressure the thickness of the material and of the bat 30 can be gaged and predetermined, according

to the uses to which my invention may be put or applied.

My wadding has many valuable characteristics due to inherent qualities of the fiber and of the pulp, and the combination, as described of the two, viz, it is light, fluffy,—even when considerably compressed,—sanitary, odorless, pliable, has a high degree of tensile strength, and has great warmth-giving qualities when sufficiently compacted as 40 a lining or filling.

My wadding and the bats formed therefrom are especially adapted for linings and fillings for various parts of automobile bodies and other upholstery purposes.

Having thus described my invention, what I claim and desire to secure by Letters Patent is:

1. A wadding composed of granular wood pulp intermixed with long cotton fiber, the latter being in the majority and forming a binder to make a substantial fabric.
2. A wadding composed of granular wood pulp intermixed with long cotton fiber, the latter being in the majority and forming a binder to make a substantial fabric, and a surface coating of glucose to produce a smooth glazed effect.

JOSEPH GATTI.